

Sept. 3, 1935.

J. P. FOSTER

2,013,042

PROCESS AND APPARATUS FOR PREPARING CELLULOSE FIBERS

Filed Feb. 5, 1934

2 Sheets-Sheet 1



John P. Foster

By Ritter, Meeklen & O'Keilly  
Attorneys

Sept. 3, 1935.

J. P. FOSTER

2,013,042

# PROCESS AND APPARATUS FOR PREPARING CELLULOSE FIBERS

Filed Feb. 5, 1934

2 Sheets-Sheet 2



Inventor

John P. Foster

By Ritter, Maclellan & O'Neill  
Attorneys

## UNITED STATES PATENT OFFICE

2,013,042

PROCESS AND APPARATUS FOR PREPARING  
CELLULOSE FIBERS

John P. Foster, Pala, Territory of Hawaii

Application February 5, 1934, Serial No. 709,880

19 Claims. (Cl. 92—9)

This invention relates to processes and apparatus for preparing useful cellulose fibers from bagasse and vegetable grasses of like character, and it comprises processes wherein the alpha cellulose fibers in bagasse are liberated by treating the bagasse in sequence first with a weak alkali, then with a dilute nitric acid solution, and finally with a stronger alkali, suitable washing steps being interposed between and following these treatments; it further comprises cyclic processes wherein a plurality of batches of bagasse are subjected to the aforesaid treatments, as will be more fully described; and it further comprises an advantageous type of beater, for use in treating the bagasse with the above chemicals, the beater being one which avoids drastic mechanical attack on the bagasse and its contained fibers, and hence permits of high yields of alpha cellulose.

The present invention, in its broadest aspect, has for its object the recovery of industrially useful cellulose fibers from bagasse. Such fibers can be used in the manufacture of paper, paper board, and similar felted fibrous materials. They may also be used in place of alpha cellulose fibers derived from other sources, such as wood pulp. My invention, therefore, relates to the liberation of such cellulose fibers from sugar-cane bagasse and grasses of like nature.

Bagasse is a waste material produced in large quantities in the recovery of sugar therefrom. There have been various proposals for the utilization of the bagasse. These are generally of two kinds. One involves the utilization of the bagasse as such for the manufacture of building boards and the like. The second proposal is directed to methods by which the ultimate cellulose fiber in the bagasse can be isolated and recovered for use in paper-making and generally as a substitute for cellulose fibers from other sources.

There is perhaps no cheaper or more abundant source of cellulose than sugar-cane bagasse. In Hawaii, for instance, the cane crop is harvested at an age of about eighteen months; in Louisiana, its age is about eight months. Great quantities of bagasse are available in every crop and the time from planting to harvesting is many times less than most other commercial sources of cellulose with the exception of cotton. Accordingly, any satisfactory method of recovering cellulose fibers in useable form from the bagasse is of very real commercial significance.

Methods to this end have been proposed hitherto. In some instances the bagasse is subjected to severe and drastic digestion with alkalis. Most

of these methods, however, do not fully take into account the very great differences between bagasse and other sources of cellulose, such as wood. Bagasse is perhaps unique among the cellulose-yielding plants and methods of removing the in-crusting substances which bind the individual fibers must take note of the character of these substances.

Bagasse contains in addition to the lignins, considerable quantities of sucrose, pentosans and similar carbohydrates. Heavy treatment with alkaline fiber-liberating reagents, for example in ways analogous to the liberation of cellulose from wood, converts the carbohydrates to gelatinous compounds which are difficult to remove from the pulp. If the alkali treatment is drastic, some of the available cellulose fibers are destroyed, that is, degradation of the available cellulose occurs. Despite modifications in the alkali treatment methods hitherto employed, loss of available cellulose has been relatively large and the expense of bleaching recovered fiber has been high.

I have now found that the yield of alpha-cellulose from bagasse can be markedly increased, and the expense of bleaching such cellulose, greatly decreased provided the bagasse be treated with both alkaline and acid reagents and my process is characterized by a three stage chemical treatment involving the use of alkalis and nitric acid. I am aware that it is not new to liberate cellulose from plant materials with nitric acid, and it is not new to follow such acid treatment by an alkaline treatment, and I make no claim to this method.

My invention departs from the aforesaid process by first subjecting the bagasse to treatment with weak alkali, advantageously about a 0.5 percent solution of caustic soda. Instead of using caustic soda, I can use a 1 percent solution of sodium carbonate, or, if desired, a mixture of both caustic soda (sodium hydroxide) and the carbonate.

This preliminary treatment is a very important step in my process and effects a pronounced removal of color. The amount of actual fiber-liberating reagents required in subsequent steps is markedly decreased. The final bleaching step is much easier and requires less bleaching agent. This will be of particular significance to those skilled in the art since it is well understood that the ease and perfection of the bleaching process is the standard by which the value of the pulp-ing process is measured.

On the attached sheets of drawings I have

illustrated, in Figure 1, my invention in flow-sheet form;

In Figure 2 I have shown an advantageous beater especially useful in my process, the view 5 being a vertical cross-section;

And in Figure 3 I have illustrated a side view of the beater.

Before proceeding to describe the flow-sheet process illustrated, I shall outline my process as 10 applied to a single batch of bagasse.

A quantity of bagasse is first shredded and screened to reduce its particle size and remove dirt. The batch is then placed in a container, such as that shown in Figures 2 and 3, and a 15 quantity of an 0.5 solution of sodium hydroxide run in. The quantity should be sufficient to fully saturate the bagasse and give a fluid pulp which can be stirred or agitated. The bagasse is treated with the alkali for from one to three hours at 20 a temperature of around 160° F. and then the solution is drained off.

As stated above, much of the undesirable color bodies are removed in this step. These are substances soluble in the weak alkali under the 25 conditions of the treatment. This alkali treatment is not sufficiently drastic to materially attack the cementitious substances binding the alpha cellulose fibers. Generally the drained-off alkali is run to waste and I then wash the alkali-treated bagasse with water. This is to remove 30 adhering alkali solution.

Without removing the washed bagasse, I next steep it for two to four hours in a 2 percent solution of nitric acid, the temperature being maintained at about 160° F. The acid solution is then drained off and the bagasse again thoroughly washed with water. Now the acid-treated and washed bagasse is subjected to the action of a stronger alkali solution. I find it best to use 40 about a 5 percent solution of sodium hydroxide or sodium carbonate, or mixtures of each. The temperature during this step is reduced to about 120° F. and the time of treatment is usually from three to six hours. Following this, the alkali 45 solution is drained off, the fiber washed with water, and the aqueous washings recovered for reuse as will be more fully described.

The actual times, concentrations, and temperatures in the foregoing three chemical treatments 50 will, of course, vary somewhat, each should be correlated with the others so that optimum yields of fiber are obtained. Naturally the source of the bagasse should be taken into account. The treatment of Louisiana bagasse, which is harvested in eight months, will differ in minor details from the treatment of Hawaiian bagasse. But the essential conditions, that is, preliminary 55 weak alkali treatment, acid treatment, stronger alkali treatment, will not be modified.

After the fiber has been liberated by the above 60 three steps, the washed fiber is bleached. Various bleaches can be used. Advantageously the bleach is a 1 to 3 percent solution of calcium or other hypochlorite. Five hours time is sufficient. 65 Chlorine itself can be used and it is best to conduct the bleaching operation at atmospheric temperature. Finally the fiber is washed free of bleaching agent. The fact that the fiber can be bleached at ordinary temperature, and by 70 using such dilute concentrations of bleaching agents, is one of the marked advantages in my process. In fact, the consumption of bleaching agent is but a fifth of that hitherto necessary when other methods of fiber liberation are employed. Aside from decreased consumption of 75

bleach, the lower temperature and concentration greatly lessens the degradation and loss of available fiber. Hence the yield is higher.

These advantages are, in part, attributable to my discovery that the cementitious substances in bagasse, as well as the impurities therein are more readily removed when the hydrogen ion concentration of the fiber-liberating reagents is changed from acid to alkaline. Some of the non-cellulosic materials are more readily soluble in acid solution; others are more readily soluble in alkaline solution. In consequence the reversal in hydrogen ion concentration employed in my process is of great value in the removal of cementitious materials. 10

Moreover, the acid treatment step is so regulated by controlling temperature and concentration, that all residual sugars in the bagasse are hydrolyzed and removed before subjecting the bagasse to an alkaline treatment strong enough 15 to convert the sugars to difficultly removable gelatinous materials. The temperature of the alkaline fiber-liberating treatment (following the acid treatment) is also so low that little of the alpha cellulose hydrolyzes, or is converted to 20 hydrated cellulose. Hence no loss of cellulose is met with. On the other hand, single treatment with acid alone, or alkali alone, would have to be far more drastic than that described herein in order to get the same degree of purification. 25 But such drastic treatment would destroy much of the available cellulose. 30

While I have more specifically referred to the use of caustic soda solutions of 0.5 percent and 5 percent strength, it is to be understood that I am not limited to these exact concentrations. In the preliminary treatment, the caustic soda can vary from about 0.5 to 1.5 percent and that used in the third step can vary from about 4 to 8 percent. Likewise the concentration of the 40 nitric acid can vary from about 1.5 to 4 or 5 percent.

Likewise the temperatures recited are merely 45 illustrative and should be varied depending upon the character and source of the bagasse. Usually a temperature of around 160° F. is best for the first alkali treatment and a somewhat lower temperature for the second alkali treatment. All temperatures given above can vary from 10° to 20° F. above or below those recited. 50

I have broadly described my invention in connection with the treatment of a single batch of bagasse. I now refer to Figure 1 on the attached drawings and will describe a commercial 55 installation of my process as adapted to the treatment of a plurality of batches.

On this figure, A, B, C, D and E are five containers for bagasse. These containers are advantageously of the type to be subsequently described. The drawing also indicates a weak soda 60 solution storage, the nitric acid storage, the stronger soda storage, water storage and bleaching solution. All of these have legends on the drawing for simplification in understanding it. Five pumps, labelled 1, 2, 3, 4 and 5 serve to pump 65 liquids from the various storage tanks to the bagasse containers or beaters.

Each beater is provided with an agitator or propeller, a screen as shown in dotted lines, and other elements as described later on. For simplification these details have been omitted in the flow-sheet. 70

In the operation of the apparatus set up illustrated (and it will, of course, be understood that the number of beaters can be increased or de- 75

creased as desired), beater A is filled with fresh, shredded and screened bagasse. Pump 4 is started and weak sodium hydroxide or sodium carbonate or a mixture of sodium hydroxide and sodium carbonate is pumped through heater 1 to the beater A until the solution reaches the desired level in the latter, at which time the run-off in the bottom of beater A is opened into the weak soda storage and adjusted to maintain a constant level of liquid in the beater, the weak soda thus circulating through beater A in a closed cycle. Heater 1 is best heated by steam coils, not shown, and serves to elevate the temperature of the solution to around 160° F. Alternatively, the beater can be provided with a heating coil, as illustrated in Figures 2 and 3, but ordinarily a separate heater will do.

As the bagasse will float in the circulating solution, it will be found desirable to start the propeller rotating so that the bagasse will be drawn down into the center of the beater. After a suitable time, as described above in connection with the treatment of a single batch of bagasse, the propeller and the circulation of solution is stopped and the weak solution is drained off to storage or to the gutter. This drained off solution will be heavily charged with coloring matter, pith fragments, dirt, etc., so it is best to discard the solution.

Then the piping connections, illustrated by lines and cross-overs on the drawing are changed so that weak soda is circulated through beater B which has meanwhile received a charge of bagasse. The procedure with B is the same as with A. After weak soda has drained from A, pump 4 is started and warm water (heated by heater 4) is circulated through the bagasse in A. Washing is continued until the water runs clear and all wash water is run to the gutter or discarded.

Piping connections are then again changed and nitric acid from its storage tank is circulated through the washed bagasse in beater A by means of pump 3, the acid being heated in heater 3 to about 160° F. After the acid treatment, the bagasse is again washed with water, the first water washings being sent to an acid recovery plant not shown. Finally, when the water washings indicate that adhering acid has been removed, pump 3 is started, and 5% sodium hydroxide circulated through heater 3 (where it is heated to about 120° F.) and beater A.

After the strong alkali treatment, the fiber in A is again washed and, by opening valves (not shown) in the various pipe lines indicated diagrammatically, the first water washings are caused to flow to the weak soda storage. In this way some of the adhering caustic soda is recovered for reuse.

The liberated fiber is then bleached with bleaching solution pumped from its storage tank by pump 5 and the fiber finally washed again with water pumped by pump 4.

Meanwhile, the bagasse in beater B has been going through a similar sequence of process steps and beaters C, D and E have also received charges of bagasse. Thus, assuming all beaters are charged, when the charge in beater E is being bleached, that in D is receiving strong soda treatment, that in C is being treated with acid, that in B is being treated with weak soda solution, and the liberated fiber in A, which has received its final water wash after the bleaching operation, is being discharged from A through a pulp outlet

schematically shown at the bottom of the screen indicated by dotted lines.

I have purposely avoided confusing the drawing with many reference characters. It will be understood that the various pipe lines are provided with suitable valves to control the flow of liquids from the various storage tanks and the drawing is simply intended to illustrate one advantageous way of carrying out my process on a large scale using a plurality of beaters.

I shall now describe an advantageous form of beater to be used in connection with my process.

In conventional pulping processes, it is customary to subject the cellulosic material, after digestion, to the action of beating engines. The well known Jordan engine is an example. These devices break down the fiber bundles thereby freeing the fibers. Not only do the engines consume much power, but their severe mechanical attack on the fibers tends to form hydrated cellulose which in turn is more readily hydrolyzed and broken down. This effect is even more pronounced in the case of relatively soft material such as bagasse.

Accordingly, I have devised a beating engine especially useful in connection with the treatment of bagasse as described above since, when using it, the hydration and consequent degradation of the cellulose fibers is reduced to a minimum. This of course means an increased yield of alpha cellulose.

In my device, I do not subject the fibers to mechanical attrition by, and contact with, mechanical "runners" or grinding wheels. I obtain a breaking down of the fiber bundles by subjecting a liquid slurry or suspension of the fibers to violent agitation whereby the beating of the material is accomplished by the impact of the bagasse particles on each other, and by the movement of the suspending liquid. This suspending liquid will invariably have a rate of speed different from that of the bagasse particles and will assist in tearing the particles apart and freeing the fibers.

Referring to Figures 2 and 3 of the drawings, the beater preferably employed in the process heretofore described comprises a metal tank 10 having a substantially cylindrical main body portion 11 and a conical bottom 12. Disposed within the tank is a perforated container 13, which may advantageously be formed of screening. The container, which is of substantially the same shape as the tank, has a cylindrical body portion 14 and a conical bottom 15 respectively spaced from the corresponding parts of the tank.

The lower end or apex of the conical bottom 15 of the container is provided with a rigid metal cap 16 having a centrally disposed discharge opening 17. The cap 16 forms convenient means to which bracing elements 18, which are rigid with the conical bottom 12 of the tank, may be attached for supporting the container within the tank in spaced relation to the latter.

Disposed within the annular space 19 between the body portions of the tank and receptacle is a heating coil 20 for receiving any suitable heating medium or fluid, such as steam. Communicating with the heating coil are suitable inlet and outlet pipes 21 and 22, respectively, in which are disposed valves 23 for controlling the passage of the heating fluid.

Extending downwardly into the beater is a rotatable shaft 24 having propeller blades 25,

which are preferably disposed adjacent the bottom of the container 13. The blades are preferably mounted in a manner, not shown, such that their pitch may be adjusted. Rotation may be imparted to the shaft 24 and consequently the propeller blades 25 by any convenient means, such as an electric motor 26, which may be supported above the beater by suitable framework designated by the reference character 27. The amount of power required to rotate the propeller will depend upon various factors, such as the density of the suspension, the speed and diameter of the propeller and the pitch and number of blades employed. It has been found that the power required to start the suspension in suitable motion is approximately one horse power per one hundred gallons, but, after the suspension is once in motion, considerably less power is required to maintain it in motion. Best results have been obtained in using the beater by so adjusting the pitch of the propeller blades and their speed (revolutions per minute) that the propeller will draw the suspension down the center of the tank, forming a funnel-shaped vortex extending downwardly to between one-half and two-thirds of the depth of the suspension. This vortiginous motion will be found to assume a compound character; that is to say, the suspension will be not only in circulation horizontally but also in circulation downwardly at the center and upwardly adjacent the periphery and at an angle which is the resultant of the two forces simultaneously applied. It is to be understood that my invention is not limited to this particular type of circulation as, in some of the operations intended to be performed by the beater, it is desirable to have a horizontal circulation or a circulation tending to the horizontal. To support the lower end of the rotatable shaft 24 and prevent it from vibrating, its lower end is preferably journaled in a bearing 28. This bearing has radiating arms 29, which are rigidly secured to the metal cap 16 of the container. Immediately above the discharge opening 17 of the cap, the shaft is preferably provided with a clearance blade or blades 30 to restrict the discharge opening and thereby prevent large articles from becoming lodged in the latter.

Communicating with the lower end of the tank 11 and the discharge opening 17 of the metal cap 16 are suitable valved passageways 31 and 32, respectively. The suspension liquid passing through the perforations of the container is adapted to be drained from the tank through the passageway 31, while the material retained within the container is adapted to discharge through the passageway 32.

From the foregoing, it will be perceived that the beater thus described is particularly advantageous for use in the treatment of bagasse and other vegetable grasses of like character.

Having thus described my invention, what I claim is:

1. The process of treating bagasse which comprises subjecting the bagasse to the action of a weak alkaline solution, then subjecting it to the action of a dilute nitric acid solution, and then subjecting it to the action of an alkaline solution stronger than that first employed.
2. The process of treating bagasse which comprises treating the bagasse with an alkaline solution equivalent in strength to approximately a 0.5 per cent solution of caustic soda at moderately elevated temperature, then treating the bagasse with a dilute nitric acid solution, and

then treating the bagasse with a solution of caustic soda stronger than that used in the first step.

3. The process as in claim 2 wherein the nitric acid solution has a concentration of about 2 percent.

4. The process of treating bagasse to liberate alpha cellulose therefrom which includes, as a preliminary step, treating shredded bagasse prior to fiber liberation with a weak alkaline solution at a moderately elevated temperature but below the boiling point, the alkaline solution being of the order of caustic soda having a concentration of about 0.5 to 1.5 percent, washing the thus treated bagasse, and then treating it with fiber-liberating reagents.

5. The process as in claim 4 wherein the caustic soda has a temperature of about 160° F.

6. The process of treating bagasse which comprises treating the bagasse with a weak caustic soda solution having a concentration of the order of 0.5 percent, washing the bagasse, treating it with a dilute nitric acid solution, washing the bagasse, treating it with a caustic soda solution having a concentration of the order of about 5 percent, washing the bagasse, and finally bleaching.

7. The process as in claim 6 wherein the nitric acid has a concentration of the order of two percent.

8. The process as in claim 6 wherein the acid and alkali treatments are conducted at moderately elevated temperatures.

9. The process as in claim 6 wherein the temperature of the first alkali treatment is about 160° F., the acid treatment about 160° F. and the second alkali treatment about 120° F.

10. The process of treating bagasse which comprises providing a plurality of batches of bagasse each batch being maintained in a separate treating receptacle, and subjecting each batch of bagasse to a sequence of steps wherein the bagasse is first treated with an alkaline solution of the order of 0.5 percent caustic soda solution, then washed with water, then treated with dilute nitric acid solution having a concentration of the order of 2 percent, then washed with water, then treated with a caustic soda solution having a concentration of the order of 5 percent, then washed with water, and finally bleaching the liberated fibers and washing free of bleaching agent, the water washings resulting from the washing of the bagasse after treatment thereof with the 5 percent caustic soda solution being used for the first alkali treatment of subsequent batches of bagasse.

11. The process of liberating alpha cellulose from bagasse which comprises first subjecting the bagasse to preliminary purification and removal of color bodies by treating the bagasse with a very weak alkali solution and then subjecting the thus treated bagasse to a fiber-liberation treatment wherein the bagasse is treated with nitric acid and then with caustic soda.

12. The process of liberating alpha cellulose from bagasse which comprises first subjecting shredded and screened bagasse to the action of a weak alkaline solution at a moderately elevated temperature but below the boiling point prior to fiber liberation to remove color bodies without materially attacking the cementitious substances binding the alpha cellulose fibers, and then subjecting the thus treated bagasse to a fiber-liberation treatment and bleaching the alpha cellulose fiber thus obtained.

13. The process of liberating alpha cellulose from bagasse which comprises first subjecting shredded and screened bagasse to a preliminary treatment with a weak solution of caustic soda to effect removal of color bodies, dirt and pith, without substantially attacking the cementitious substances binding the alpha cellulose fibers, and then subjecting the thus treated bagasse to the action of a dilute nitric acid solution, and a dilute caustic soda solution to liberate alpha cellulose, washing the treated fibers after the acid and alkali treatment, and utilizing the wash water from said dilute alkali treatment to preliminarily treat further quantities of bagasse.

14. The process of treating bagasse to liberate alpha cellulose therefrom which includes, as a preliminary step prior to fiber liberation, treating the shredded bagasse with a weak alkali solution at a moderately elevated temperature but below the boiling point to effect removal of color bodies, pith, and dirt whereby subsequent bleaching of the liberated alpha cellulose is facilitated and the consumption of bleaching agent reduced.

15. A beater for the treatment of bagasse and the like involving a tank, a perforate container disposed within the tank in spaced relation thereto, heating elements in the space between said tank and the container, and a rotatable shaft extending downwardly into said container to near the bottom thereof, said shaft being provided with a propeller device adjacent its lower end and said tank and container having individually controlled discharge outlets.

16. A beater for the treatment of bagasse and the like involving a tank having a conical bottom, a perforate container also having a conical bottom disposed within the tank in spaced relation to the latter, the lower end of said container having a rigid cap, a rotatable shaft extending downwardly into said container and provided with propeller blades adjacent its lower end, means rigid with said cap affording a bearing for the lower end of said shaft, and discharge outlets respectively located in the lower ends of said tank and container.

17. A beater as described in claim 16 having heating elements in the space between the tank and container.

18. A beater for the treatment of bagasse and the like involving a tank having a conical bottom, a perforate container disposed within the tank and having a conical bottom spaced from the bottom of the tank, the lower portion of the conical bottom of the container being provided with a rigid cap having a central discharge opening, means rigid with said cap for supporting the container in spaced relation to the tank, and a rotatable shaft extending downwardly into said container provided with a propeller device disposed adjacent the bottom of the container.

19. A beater as described in claim 18, in which the lower end of the rotatable shaft is provided with means spaced above the discharge opening of the cap for restricting said opening.

JOHN P. FOSTER.